

3,451,930  
LUBRICANT COMPOSITION FOR HIGHLY  
STRESSED GEARS

George A. Mead, Scotch Plains, N.J., assignor to Esso  
Research and Engineering Company, a corporation of  
Delaware  
No Drawing. Filed Sept. 16, 1966, Ser. No. 579,833  
Int. Cl. C10m 3/42  
U.S. Cl. 252—32.7

4 Claims

## ABSTRACT OF THE DISCLOSURE

A lubricating oil composition capable of satisfactory lubrication of gears subjected to very high loads consists of a major proportion of a lubricating oil base and a minor proportion of a synergistic mixture of an alkaline earth metal salt of a hydrocarbon sulfonic acid, a Group II metal salt of a dialkyl dithiophosphoric acid, and a halogenated hydrocarbon of from 35 to 75 weight percent halogen content.

This invention concerns an improved lubricating oil composition which is particularly useful in mechanical systems, wherein the gears are under high stresses as, for example, in rear axles and in tractor transmissions. In particular the invention concerns a gear lubricant containing in combination an alkaline earth metal salt of a hydrocarbon sulfonic acid, a metal salt of a dialkyl dithiophosphoric acid and a chlorinated hydrocarbon.

There are many modern day mechanical systems wherein a lubricant must serve both as a transmission fluid and as a gear lubricant. One such system is what is known as a transaxle unit wherein the transmission and the rear axle system of an automobile are combined into a single mechanical unit located near the rear wheels of the automobile. Another such system is the transmission of a modern farm tractor. In such mechanical systems the gears are placed under high stress and thus require a lubricant which will perform satisfactorily.

In accordance with the present invention it has been found that an unusually effective gear oil composition capable of satisfactory lubrication under conditions wherein the gears are under very high loads, e.g. 500,000 pounds per square inch, can be prepared by incorporating into the composition a combination of three types of additives. One of these is an alkaline earth metal salt of a hydrocarbon sulfonic acid having a molecular weight in the range of about 400 to 900. A second component is a metal salt of a dialkyl dithiophosphoric acid and the third component is a chlorinated hydrocarbon. Each of these additives has been employed in the past as a component of a lubricating composition. Chlorinated hydrocarbons are well known components capable of imparting extreme pressure properties to a lubricating oil. Metal salts of dialkyl dithiophosphoric acids are known in the art as anti-wear agents and as anti-oxidants. Alkaline earth metal salts of hydrocarbon sulfonic acids have been employed in the art primarily as dispersants. It has now been surprisingly found that these three types of additives in combination exert a synergistic improvement in load-carrying capacity.

The alkaline earth metal salts employed in this invention are the metal salts of hydrocarbon sulfonic acids wherein the acids have molecular weights in the range of about 400 to 900. The alkaline earth metal salts include those of calcium, strontium and barium. Sulfonic acids from which the salts are prepared are classified generally as either petroleum sulfonic acids or synthetic sulfonic acids. Petroleum sulfonic acids are produced by treating petroleum fractions, including lubricating oil distillate fractions, the so-called white oil distillates, or other pe-

roleum fractions such as petrodatum, with suitable sulfonating agents including sulfur trioxide, concentrated sulfuric acid and fuming sulfuric acid. Synthetic sulfonic acids are prepared by treating relatively pure synthetic hydrocarbons in the same manner. Usually the synthetic hydrocarbons are alkylated aromatic hydrocarbons such as the products of alkylation of benzene, toluene, xylene or naphthalene. Typically benzene is alkylated with a polymer of propylene or butylene, e.g. butylene trimer, to form a C<sub>12</sub> alkyl benzene which is then sulfonated as above-described. The natural or synthetic sulfonic acids whose alkaline earth metal salts are used in this invention include alkane sulfonic acids, aromatic sulfonic acids, alkaryl sulfonic acids, and aralkyl sulfonic acids.

The term sulfonate as used herein and in the appended claims includes both neutral sulfonates, i.e. those wherein the sulfonic acids have been neutralized with an equal mole equivalent of metal base, and high alkalinity sulfonates wherein additional metal base in excess of that required for simple neutralization has been reacted with the sulfonic acids to form an alkaline product which is then normally blown with an acidic gas such as CO<sub>2</sub>. Overbased or high alkalinity sulfonates can have base numbers of from 30 to as much as 350. Base number is defined in numerical terms equivalent to milligrams of KOH per gram of the material. It is preferred to employ in the present invention an alkaline earth metal sulfonate having a total base number of at least 60 and more preferably one having a total base number of from about 200 to 350 in order to impart rust inhibiting properties to the composition. Specific examples of alkaline earth metal sulfonates that can be employed in the present invention include a barium petroleum sulfonate of about 950 molecular weight, calcium C<sub>8</sub> alkyl benzene sulfonate (from benzene alkylated with diisobutylene), barium C<sub>16</sub> alkyl benzene sulfonate (from benzene alkylated with tetraisobutylene), calcium petroleum sulfonate of about 880 molecular weight, calcium salt of sulfonated bottoms from C<sub>12</sub> alkyl benzene (C<sub>12</sub> group from tetrapropylene) overbased to 200 base number, a barium salt of 560 molecular weight petroleum sulfonic acids and the calcium salts of petroleum sulfonic acids of about 450 molecular weight overbased to a base number of about 225.

The metal salts of dialkyl dithiophosphoric acids are well known in the art. It is common practice to prepare dialkyl dithiophosphoric acids by reacting phosphorus pentasulfide with an aliphatic alcohol or a mixture of aliphatic alcohols containing the desired range of alkyl groups in a molar ratio of approximately 4 moles of alcohol for each mole of phosphorus pentasulfide. The acids are then neutralized with an oxide, hydroxide or carbonate of a polyvalent metal, or alternatively with a reactive polyvalent metal salt. The present invention employs polyvalent metal salts of dialkyl dithiophosphoric acids prepared from alcohols having in the range of from about 3 to about 12 carbon atoms. The dialkyl dithiophosphoric acids whose salts are used in this invention include not only those made from a simple aliphatic alcohol such as isopropyl, normal butyl, normal decyl, etc., but also from mixed aliphatic alcohols including the C<sub>5</sub> or C<sub>8</sub> alcohols obtained by reaction of olefins with carbon monoxide and hydrogen and subsequent hydrogenation of the resultant aldehydes. Also there can be used dithiophosphoric acids obtained from such mixtures as isopropyl alcohol mixed with methyl isobutyl carbinol, a combination of primary amyl alcohol and isobutanol, a combination of mixed amyl alcohols and technical lauryl alcohol, a mixture of isopropyl alcohol and C<sub>8</sub> Oxo alcohol, and the like. Mixed acids obtained by reaction of individual alcohols separately with P<sub>2</sub>S<sub>5</sub> can also be employed in the preparation of the metal salts. The metals employed in making the salts are those of Group II of the Periodic Table including

zinc, cadmium, barium and magnesium. Zinc salts are particularly preferred.

The halogenated hydrocarbons employed in the present invention are preferably chlorinated hydrocarbons, although iodinated, fluorinated, or brominated hydrocarbons may also be used. The halogenated hydrocarbons will have a halogen content within the range of about 35 to 75 wt. percent, or more preferably from 40 to 70 wt. percent. The hydrocarbons that are halogenated will have carbon contents ranging from about C<sub>8</sub> to C<sub>24</sub>. The halogenated hydrocarbons are produced through the direct halogenation of the hydrocarbons or by other known means. In the case of chlorinated hydrocarbons it is ordinarily necessary only to bubble the chlorine through the hydrocarbon in the liquid state. For example, paraffin wax can be heated to a temperature in the range of about 150° to 200° F. and chlorine bubbled through it until the desired amount of chlorine has been introduced. Iodination of hydrocarbons is taught in U.S. Patent 3,184,413. The hydrocarbons that are halogenated include aliphatic hydrocarbons and terpenes. Chlorinated paraffin wax is particularly preferred, e.g. a paraffin wax of 122° F. melting point that has been chlorinated to 40% chlorine content or a paraffin wax of 130° F. melting point that has been chlorinated to 50% chlorine content. Other examples include chlorinated kerosene of 42% chlorine content, chlorinated polyisobutylene of 850 molecular weight containing 47% chlorine, fluorinated petrolatum containing 55% fluorine, and iodinated polyisobutylene of 780 molecular weight containing 70 wt. percent iodine. Polyhalogenated isoparaffins may also be used, including 2,5-dichloro-4-chloromethyl-2,4-dimethyl pentane and 1,4,5-trifluoro-2,2,4-trimethyl pentane.

The base oil used in compounding the gear oils of this invention will include any of the base oils that are conventionally employed for this service and can thus vary widely in refinement, type and viscosity. They can be derived from a variety of crudes including paraffinic, naphthenic, asphaltic or mixed base and they can be treated by any of the conventional refining methods including hydrogen treating, acid treating extraction, etc. In general, the viscosity will be in the range of from about 60 to 3500 SUS at 100° F., or more usually in the range of about 100 to 2000 SUS at 100° F. Synthetic lubricating oils may be employed in addition to mineral lubricating oils.

The gear oils of this invention can also contain, in addition to the combination of additives described above, other additives for their known functions including anti-foam agents, rust inhibitors, corrosion inhibitors, demulsifiers, metal deactivators, pour point depressants and the like either singly or in combination.

The additive combination of the present invention will be employed in the gear oil composition within the concentration ranges set forth below:

|                                                                    | Weight percent concentration |           |
|--------------------------------------------------------------------|------------------------------|-----------|
|                                                                    | Broad                        | Preferred |
| Metal sulfonate                                                    | 0.3-4                        | 0.5-3     |
| Metal dialkyl dithiophosphate                                      | 0.2-3                        | 0.8-2     |
| Halogenated hydrocarbon sufficient to furnish halogen in amount of | 0.2-3                        | 0.8-2     |

The weight percents given are on the basis of the total composition. In the above combination of additives the

The invention will be better understood when reference is made to the following examples which include a preferred embodiment:

#### Example 1

A number of gear oil compositions were prepared using as the base oil a solvent refined neutral lubricating oil having a viscosity of 450 SUS at 100° F. The three additive components that were employed were a chlorinated constituent not less than 15 wt. percent of the entire combination of the three types of additives.

10 ingredient that is present in the least concentration should paraffin wax of 50% chlorine content, a zinc dialkyl dithiophosphate and an overbased calcium sulfonate. The chlorinated wax was a purchased material having a viscosity of 200 SUS at 210° F., and a specific gravity of 128 at 60° F. (10.6 lbs. per gallon). The overbased calcium sulfonate was a purchased material which was a concentrate in mineral oil of a calcium sulfonate derived from synthetic alkylated aromatic hydrocarbons wherein the sulfonic acids averaged about 420 molecular weight. The concentrate contained 11.4% calcium, representing approximately 30 wt. percent calcium sulfonate and 24 to 25 wt. percent CaCO<sub>3</sub>. The total base number was about 300 milligrams of KOH per gram. The zinc dialkyl dithiophosphate was also a purchased material which consisted of an oil solution containing about 25 wt. percent of mineral lubricating oil and about 75 wt. percent of zinc dialkyl dithiophosphates derived from the treatment of a mixture of isobutanol and mixed amyl alcohols with P<sub>2</sub>S<sub>5</sub> followed by neutralization with zinc oxide.

15 Each of the gear oil compositions was prepared by simple mixing of the additives with the lubricating oil base. In some of the compositions only one additive was employed in other compositions two of the additives were employed, and in a third set of compositions all three of the additives were employed. The load-carrying ability of 20 each of the compositions was determined using the Mean Hertz Load Test.

25 The Mean Hertz Load Test is designated as Method 6503.1 of Federal Test Method Standard No. 791a, dated July 27, 1964. Briefly described it involves use of the well-known 4-ball extreme pressure test apparatus (also called the Shell 4-ball test machine) wherein a steel ball held in a check is pressed against three other steel balls 30 fixed in position by a screw cap, and the first ball is rotated against the other balls under set conditions of force, temperature and speed of rotation. In this particular test the force is gradually increased until welding occurs. Then the scars on the steel balls are measured, and the 35 mean load is calculated from those measurements.

The ingredients in each of the compositions tested and the test results expressed as the Mean Hertz Load, kg., are given in the following Table I. The concentration of each of the additives in the table is the actual amount 40 that was present, ignoring the diluent oil when such was present in the additive as supplied.

TABLE I

| Composition, wt. percent | Base oil | Blend |      |      |      |      |      |      |      |      |      |      |
|--------------------------|----------|-------|------|------|------|------|------|------|------|------|------|------|
|                          |          | A-1   | A-2  | B-1  | B-2  | C-1  | C-2  | D    | E    | F    | G-1  | G-2  |
| ZDDP <sup>1</sup>        |          | 1.5   | 3.0  |      |      |      |      | 1.5  | 1.5  |      | 1.5  | 1.5  |
| Sulfonate <sup>2</sup>   |          |       |      | 1.0  | 2.0  |      |      | 2.0  |      | 2.0  | 2.0  | 1.0  |
| Chlorinated wax          |          |       |      |      |      | 3.0  | 6.0  |      | 3.0  | 3.0  | 3.0  | 3.0  |
| Base oil <sup>3</sup>    | 100      | 98.5  | 97.0 | 99.0 | 98.0 | 97.0 | 94.0 | 96.5 | 95.5 | 94.0 | 93.5 | 94.5 |
| Mean Hertz load, kg.     | 20.3     | 42.5  | 42.3 | 36.3 | 32.3 | 32.8 | 26.0 | 40.7 | 41.8 | 38.3 | 52.0 | 47.3 |

<sup>1</sup> Zinc dialkyl dithiophosphates.

<sup>2</sup> Includes overbasing components as well as sulfonate itself, but not diluent oil.

<sup>3</sup> Includes oil present in additive concentrate, where applicable.

It will be noted from the test results in Table I that the addition of 1.5 wt. percent of zinc dialkyl dithiophosphate to the base oil produced a significant increase in the Mean Hertz Load, i.e. from 20.3 kg. to 42.5 kg. However when the amount of this additive was doubled to 3 wt. percent there was no further increase in Mean Hertz Load (Blends A-1 and A-2). It is also noted that the addition of 1 wt. percent of the overbased calcium sulfonate to the same base oil produced a significant increase in Mean Hertz Load from 20.3 kg. to 36.3 kg. Here again doubling the quantity of the additive in the base oil did not result in any further increase in Mean Hertz Load (Blends B-1 and B-2). The addition of 3 wt. percent of chlorinated wax containing 50 wt. percent chlorine produced a significant increase in the load reading, from 20.3 kg. to 32.8 kg. However, when the quantity of this additive was doubled there was no further increase in Mean Hertz Load (Blends C-1 and C-2).

Looking now at the results obtained when combinations of two of the three ingredients were employed, it will be noted that there was no increase in the Mean Hertz Load when 2 wt. percent of the overbased calcium sulfonate was added to the composition that contained 1.5 wt. percent of the zinc dialkyl dithiophosphate (Blend D) nor when 3 wt. percent of chlorinated wax was added to the blend containing 1.5 wt. percent of zinc dialkyl dithiophosphate (Blend E). While the addition of 2 wt. percent of overbased calcium sulfonate to the oil composition that contained 3 wt. percent of chlorinated wax (Blend F) resulted in some improvement in the load reading, i.e. from 32.8 kg. to 38.3 kg., the value reached was not as high as that when 1.5 wt. percent of zinc dialkyl dithiophosphate was used alone, i.e. 42.5 kg. (Blend A-1).

Referring now to the compositions wherein all three of the components were present, it will be noted that a combination of 1.5 wt. percent of zinc dialkyl dithiophosphate, 2 wt. percent of the overbased calcium sulfonate and 3 wt. percent of chlorinated wax gave a Mean Hertz Load of 52.0 kg. (G-1), which is higher than would be expected by doubling the concentration of the individual additives or by adding one of the additives to the composition containing just one of the other additives. Similarly, one-half as much of the calcium sulfonate was employed in the composition containing all three components (G-2). A load reading of 47.3 kg. was obtained. Thus there was a surprising synergy in the load-carrying ability of the composition when all three of the additives were present.

#### Example 2

Additional blends were prepared employing the same base stock, the same chlorinated wax and the same zinc dialkyl dithiophosphate as described in Example 1 but different metal sulfonates. One of these was a 45 wt. percent concentrate in oil of a neutral calcium petroleum sulfonate derived from 450 molecular weight petroleum sulfonic acids. The other was a 45 volume percent concentrate of a high alkalinity barium synthetic sulfonate derived from alkyl benzene sulfonic acids of about 460 molecular weight. The concentrate analyzed 14.5% barium and had a total base number of about 59. Blends containing all three ingredients, i.e. either of the sulfonates just described along with the zinc dialkyl dithiophosphate and the chlorinated wax, were compared with other blends containing only either of the described sulfonates. The Mean Hertz Load data that were obtained and the compositions of each of the blends are given in the following Table II. Here again, the actual concentration of each additive is given, ignoring the diluent oil.

6  
TABLE II

| Composition, wt. percent   | Blend |      |      |      |
|----------------------------|-------|------|------|------|
|                            | H     | J    | K    | L    |
| ZDDP <sup>1</sup>          |       |      |      |      |
| Chlorinated wax            |       |      | 1.5  | 1.5  |
| Neutral calcium sulfonate  |       | 3.0  | 3.0  |      |
| Overbased barium sulfonate | 1.2   |      | 1.2  |      |
| Base oil <sup>2</sup>      | 98.8  | 98.8 | 94.3 | 94.3 |
| Mean Hertz load, kg.       | 25.5  | 21.2 | 46.7 | 45.8 |

<sup>1</sup> Zinc dialkyl dithiophosphates.

<sup>2</sup> Includes oil from concentrates.

#### Example 3

A gear oil blend suitable for use in the present invention is prepared by blending together 73.3 wt. percent of the base oil described in Example 1, 17.4 wt. percent of solvent-deasphalted, solvent-dewaxed Mid-Continent residuum of about 207 SSU viscosity at 210°F., 0.5 wt. percent of a pour point depressant comprising wax-alkylated naphthalene, 2.0 wt. percent of a 70 wt. percent concentrate of zinc dialkyl dithiophosphates in lubricating oil, said dialkyl dithiophosphates being derived from a mixture of  $P_2S_5$  treated isopropyl alcohol and  $P_2S_5$  treated methylbutyl carbinol, 3.0 wt. percent of a chlorinated kerosene of 41% chlorine content and 4.0 wt. percent of an overbased calcium sulfonate concentrate comprising 42 wt. percent of diluent oil and the balance the overbased additive. The base number of the calcium sulfonate concentrate is 250 and the calcium sulfonate is derived from petroleum sulfonic acids of about 450 molecular weight.

#### Example 4

A gear oil composition was prepared by simple mixing of 74 wt. percent of the base oil described in Example 1, 17.5 wt. percent of the residuum described in Example 3, 0.5 wt. percent of the pour point depressant described in Example 3, 1.0 wt. percent sorbitan monooleate rust inhibitor, 2.0 wt. percent of calcium sulfonate concentrate, 3.0 wt. percent of chlorinated paraffin wax and 2.0 wt. percent of zinc dialkyl dithiophosphate concentrate, those last three additives being those described in Example 1. The Mean Hertz Load for this composition was found to be 56.4 kg.

This composition was used to lubricate a farm tractor transmission that contained all of the usual transmission gears together with the final drive gears, which included a spiral bevel pinion and ring gear. The transmission was run with this oil composition at an oil temperature of 180°F. with a load that placed 450,000 to 500,000 p.s.i. contact stress on the final drive gears. Under those conditions the run lasted for more than 200 hours before failure of the final drive gears, which was considered to be excellent performance.

Thus the compositions of this invention are particularly suitable for lubricating transmissions having gears that are subjected to contact stresses of at least 450,000 pounds per square inch.

It is not intended that the specific examples herein presented limit this invention in any manner.

What is claimed is:

1. An improved lubricating oil composition capable of serving both as a transmission fluid and as a lubricant for gears subjected to high stresses, which consists essentially of a major proportion of a lubricating oil base and a minor proportion of a load-carrying additive combination of:
  - A. an alkaline earth metal salt of a hydrocarbon sulfonic acid having a molecular weight within the range of about 400 to 900;
  - B. a zinc salt of a dialkyl dithiophosphoric acid wherein the alkyl groups are within the range of 3 to 12 carbon atoms; and
  - C. chlorinated paraffin wax having from 35 to 75 weight percent chlorine;
- each of said components A, B, and C constituting

at least 15 weight percent of the total of A plus B plus C; there being present in said lubricating oil composition, based on the total composition, from about 0.3 to 4 weight percent of A, from about 0.2 to 3 weight percent of B, and from about 0.5 to 10 weight percent of C; the amount of C that is present in said lubricating oil composition being such as to impart to said composition from about 0.2 to 3 weight percent of chlorine.

2. Lubricant as defined by claim 1 wherein said sulfonic acid salt has a total base number of at least 60.

3. Lubricant as defined by claim 1 wherein said sulfonic acid salt is an overbased calcium sulfonate of about 300 total base number.

4. Lubricant as defined by claim 1 wherein said dialkyl dithiophosphoric acid salt is the zinc salt of mixed C<sub>4</sub>-C<sub>5</sub> dialkyl dithiophosphoric acids.

5 References Cited

UNITED STATES PATENTS

|           |         |               |       |           |
|-----------|---------|---------------|-------|-----------|
| 2,119,556 | 6/1938  | Prutton       | ----- | 252—58    |
| 2,126,590 | 8/1938  | Valentine     | ----- | 252—58    |
| 3,236,770 | 2/1966  | Matson et al. | ----- | 252—32.7  |
| 3,238,130 | 3/1966  | Matson.       |       |           |
| 3,290,347 | 12/1966 | Miller        | ----- | 260—429.9 |

PATRICK P. GARVIN, Primary Examiner.

U.S. Cl. X.R.

15 252—75